# EUROPEAN PATENT SPECIFICATION

(11) **EP 2 156 761 B1**
(45) Date of publication and mention of the grant of the patent: **31.10.2012**
(21) Application number: 09010687.3
(22) Date of filing: 19.08.2009
(51) Int. Cl.: A42B 3/06, A42C 2/00

(54) **Method for making a helmet and the helmet made thereby**
Verfahren zur Herstellung eines Helmes und danach hergestellter Helm
Méthode pour fabriquer un casque et casque ainsi fabriqué

(30) Priority: 20.08.2008 TW 97131670
(43) Date of publication of application: 24.02.2010
(73) Proprietor: Wang, Tse-Ping, Taipei City, 106 (TW)
(72) Inventor: Wang, Tse-Ping, Taipei City, 106 (TW)
(74) Representative: Schaeberle, Steffen

(56) References cited:
- US-A- 5 376 318
- US-A- 5 598 588
- US-A- 5 833 796
- US-A- 6 105 176
- US-A1- 2007 277 296

## Description

### BACKGROUND OF THE INVENTION

### Field of Invention

The invention relates to a method of manufacturing sports helmets and, in particular, to the method of manufacturing fusion in-mould helmets.

### Related Art

The structures of sports helmets, such as bicycle helmets, skate helmets, snow helmets, climbing helmets, and riding helmets, are more or less the same with a harder outer shell and a softer shock absorbing inner shell. However, higher-end helmets are integrally formed having a thin polycarbonate outer shell with the softer inner shell material injected into the outer shell so that the two parts are formed together. When impact occurs, the light harder shell and softer inner shell work together to absorb the shock. Such types of helmet are commonly called in-mould.

The above-mentioned outer helmets are usually made of costly polycarbonate. In view of the high cost of polycarbonate, manufacturers are forced to consider cheaper materials instead. In this case, PVC, PET, and PETG are substitutes see for example US 5,833,796, US 6,105,176 and US 2007/0277 296. Nevertheless, these cheaper substitutes cannot withstand high temperatures during the forming process. The forming process thus has to be done at lower temperatures. But using normal processes, when forming at lower temperatures, the outer shell and inner shell cannot bond together.

### SUMMARY OF THE INVENTION

In view of the foregoing, an objective of the invention is to provide in-mould helmet formed using lower temperatures but still creating an integral bond between the two shell materials.. Plastic shell material that cannot withstand high temperatures (such as PVC, PET, PETG and others) is first printed and then thermoformed. And then the vents and the edges are trimmed to form an outer helmet. The outer helmet is then pressed together with a pre-formed inner helmet in a molding machine. They are integrally formed into a sports helmet at lower pressure, lower temperature, and shorter time using the method of claim 1.

### BRIEF DESCRIPTION OF THE DRAWINGS

The invention will become more fully understood from the detailed description given herein below illustration only, and thus is not limitative of the present invention, and wherein:

None.

### DETAILED DESCRIPTION OF THE INVENTION

The present invention will be apparent from the following detailed description.

The invention is implemented as follows. Outer shell material that cannot withstand high temperatures (e.g., 90°C or more), such PVC, PET, and PETG, is formed on thermo vacuuming machine. Afterwards, it is made into an outer helmet after printing, plastic removal, edge cutting, hole drilling, and so on.

The PVC, PET, or PETG outer helmet thus formed is pressed together with a pre-formed inner liner (normally made from expanded polystyrene (EPS) or similar materials) in a moulding machine. They are integrally formed into a sports helmet at lower pressure (0.5±0.1 bar), lower temperature (110±2 °C), and shorter time (168±5 sec).

The fusion in-mould helmet formed according to the above-mentioned method can have the same or similar appearance, functions, collision protection, and shock absorption as the conventional expensive polycarbonate outer helmet.

According to the above-mentioned fusion in-mould helmet, there is no gap between the PVC, PET, or PETG outer helmet and the EPS inner helmet because they are integrally formed. This helps distributing the stress during a collision, thereby protecting the head.

The above-mentioned fusion in-mould helmet can prevent the problem of deformation due to direct sunlight as opposed to when the PVC, PET, or PETG outer shell is combined with the EPS inner helmet by glue or tape.

Although the invention has been described with reference to specific embodiments, this description is not meant to be construed in a limiting sense. Various modifications of the disclosed embodiments, as well as alternative embodiments, will be apparent to persons skilled in the art. It is, therefore, contemplated that the appended claims will cover all modifications that fall within the true scope of the invention.

## Claims

1. Method for producing a fusion in-mould helmet comprising
an outer helmet formed from a plastic plate, wherein the material of the outer helmet is PVC, or PET, or PETG. by printing, thermoforming, plastic removal, edge cutting, and hole drilling, **characterised in that**
the outer helmet and a pre-formed inner helmet are disposed together in a moulding machine to integrally form the in-mould helmet at lower pressure, lower temperature, and shorter time,
wherein the pressure for fusion is not more than 0.7+-0.1bar.
wherein the temperature for fusion is not more than 110+-2°C, and wherein the time for fusion is not more than 168+-5 sec.

2. The method of claim 1, wherein the material of the inner helmet is expanded polystyrene (EPS).

3. A fusion in - mould helmet produced by a method according to claim 1 or 2.

## Patentansprüche

1. Verfahren zum Herstellen eines Helmes durch Fusion in einer Form, aufweisend:
einen Außenhelm, der aus einer Kunststoffplatte durch Drucken, Thermoformen, Kunststoffentfernen, Schneiden und Lochbohren ausgebildet wird, wobei das Material des Außenhelmes PVC oder PET oder PETG ist, **dadurch gekennzeichnet, dass**
der Außenhelm und der vorgeformte Innenhelm zusammen in einer Formgebungsmaschine angeordnet sind, um den Helm in der Form bei geringerem Druck, geringerer Temperatur und kürzerer Zeit einstückig auszubilden,
wobei der Druck zur Fusion nicht mehr als 0,7 + - 0,1 bar beträgt,
wobei die Temperatur zur Fusion nicht mehr als 110 + - 2° C beträgt, und
wobei die Zeit zur Fusion nicht mehr als 168 + - 5 Sek. beträgt.

2. Verfahren gemäß Anspruch 1, wobei das Material des Innenhelmes Polystyrol schaum (EPS) ist.

3. Fusion-in-Form Helm, hergestellt durch ein Verfahren gemäß Anspruch 1 oder 2.

## Revendications

1. Procédé pour fabriquer un casque dans le moule par fusion comprenant :
un casque extérieur formé à partir d'une plaque en plastique, dans lequel le matériau du casque extérieur est du PVC, ou du PET, ou du PETG, par impression, thermoformage, élimination de plastique, coupage de bord, et perçage de trou, **caractérisé en ce que**
le casque extérieur et un casque intérieur préformé sont disposés ensemble dans une machine de moulage pour former en un seul bloc le casque dans le moule à une pression inférieure, une température inférieure et en un temps plus court,
dans lequel la pression pour la fusion n'est pas supérieure à 0,7 +-0,1 bar,
dans lequel la température pour la fusion n'est pas supérieure à 110+-2 °C, et
dans lequel le temps pour la fusion n'est pas supérieur à 168+-5 sec.

2. Procédé selon la revendication 1, dans lequel le matériau du casque intérieur est du polystyrène expansé (EPS).

3. Casque dans le moule par fusion fabriqué par un procédé selon la revendication 1 ou 2.
